

# UNITED STATES PATENT OFFICE.

OSCAR KLAUSER, OF HERISAU, SWITZERLAND, ASSIGNOR TO THE FIRM OF AKTIEN-  
GESELLSCHAFT CILANDER, OF HERISAU, SWITZERLAND.

## TREATMENT OF COTTON FABRICS.

1,258,225.

Specification of Letters Patent.

Patented Mar. 5, 1918.

No Drawing.

Application filed August 12, 1916. Serial No. 114,620.

*To all whom it may concern:*

Be it known that I, OSCAR KLAUSER, a citizen of the Republic of Switzerland, residing at Herisau, Kasernenstrasse 96 D, 5 Switzerland, have invented certain new and useful Improvements in Processes for the Treatment of Cotton Fabrics; and I do hereby declare the following to be a full, clear, and exact description of the invention, such 10 as will enable others skilled in the art to which it appertains to make and use the same.

It is a well-known fact that if treated with sulfuric acid of at least  $50\frac{1}{2}$ ° Bé., ordinary 15 cotton or cotton already mercerized will assume a parchment-like appearance by becoming transparent and somewhat stiff. These qualities may be intensified by submitting the stretched fabric to a subsequent 20 treatment with lye of  $25^{\circ}$ – $30^{\circ}$  Bé.

Now, if sulfuric acid of a lower concentration than  $50\frac{1}{2}$ ° Bé. is used at normal temperature, *e. g.*, between  $0^{\circ}$  and  $15^{\circ}$  centigrade, the effect on the fabric will be far less pronounced, only a slight, if any, transparency being imparted to the cotton. In this case 25 the action of the sulfuric acid will be a purely mercerizing one. (See Thomas and Prevost, British Patent No. 20714 of 1896). 30 According to German Patent No. 129883 (Thomas and Prevost) the action of weaker sulfuric acid may be intensified by subsequent alkali-treatment, but even then only a comparatively low degree of transparency 35 can be attained.

I have discovered that sulfuric acid of less than  $50\frac{1}{2}$ ° Bé. (measured at  $15^{\circ}$  C. above zero) has an entirely new effect on cotton, if used at a temperature of not more than  $4^{\circ}$  40 below zero. If such cold sulfuric acid is employed, a subsequent treatment with lye will have the same effect as if sulfuric acid of more than  $50\frac{1}{2}$ ° Bé. had been used at normal temperature. Thus, if cold sulfuric acid 45 of  $50^{\circ}$  Bé. is used through a period of at least five seconds or cold sulfuric acid of  $49^{\circ}$  Bé. through a period of several minutes, and if subsequently the mercerizing action of a lye is applied—the latter being preferably 50 also at a low temperature, about  $0^{\circ}$  C.—then the cotton thus treated will receive a transparent appearance.

By varying the length of time of dipping the cotton, and the temperature and concentration of the sulfuric acid employed, it is

possible to obtain fabrics of a desired degree of transparency. Owing to the very low temperature of the sulfuric acid, it is possible to keep the cotton in contact with it for a period of ten minutes and more, so 60 that there is sufficient time for the acid to thoroughly soak into the cotton fiber, so that a more uniform transparency is obtained than with the use of sulfuric acid of  $50\frac{1}{2}$ ° Bé. at normal temperature, in which 65 latter case the duration of contact between cotton and acid may not exceed 20 seconds.

If one piece of cotton fabric is first treated in sulfuric acid of  $49^{\circ}$  Bé. at  $10^{\circ}$  C. below zero and mercerized, and a second piece 70 of cotton fabric is first treated in a sulfuric acid of the same concentration but at  $15^{\circ}$  C. above zero and also mercerized, and if both pieces are then dipped into the same dye-bath, the first piece will prove to have been 75 dyed to a considerably darker color than the second piece, which is another advantage of the use of cold sulfuric acid.

If a cotton fabric is dipped, for a period of several minutes, into sulfuric acid at a 80 low temperature, then washed and dried without being stretched, the fabric will become of a wool-like appearance. Up to now, working at normal temperature, such a result could be obtained with sulfuric acid of 85  $49$ – $51^{\circ}$  Bé., only if the cotton treated had undergone a preliminary mercerization or else was subsequently submitted to the action of lye and dried without being stretched.

It is obvious that by means of suitably applied reserves, the action of the cold sulfuric acid might be localized, and patterns obtained. In this case the use of cold acid is especially advantageous, as its action on the 95 reserve coating will be less intense than could be the case with acid of higher concentration and at normal temperature, so that the resulting pattern has a clearer outline.

Thus, by using a reserve with the acid treatment and subsequent mercerization and stretching of the fabric, a pattern of transparent places on a nontransparent ground may be obtained, while if used with the acid 100 treatment alone, places of woolly appearance will result on a smooth ground.

These patterns may be dyed, when the effect will be still more enhanced, as the parts 105 of the fabric that have been under the action of the fabric that have been under the action

100

105

110

of sulfuric acid will take a deeper stain with most dyes.

Having now particularly described and ascertained the nature of the said invention 5 and in what manner the same is to be performed, I declare that what I claim is:

1. Process for the treatment of cotton fabrics, comprising subjecting the fabric to the action of sulfuric acid of less than 10  $50.50^{\circ}$  Bé., at a temperature considerably below  $0^{\circ}$  C., and subsequently treating the fabric with lye of about  $0^{\circ}$  C., and stretching it, to obtain transparency of the fabric.

2. Process for the treatment of cotton 15 fabrics, comprising subjecting the fabric to the action of sulfuric acid of less than  $50.50^{\circ}$  Bé., at a temperature considerably below  $0^{\circ}$  C., in combination with a reserve, and thereafter treating the fabric with lye 20 at a temperature of about  $0^{\circ}$  C., and stretching it to obtain transparent patterns.

3. A step in the process for the treatment of cotton fabrics, which comprises treating the fabric with a cold sulfuric acid solution of a concentration less than  $50.50^{\circ}$  Bé. 25 and below  $0^{\circ}$  C.

4. Process for the treatment of cotton fabrics, comprising subjecting the fabric to the action of sulfuric acid of less than  $50.50^{\circ}$  Bé. at a temperature considerably below  $0^{\circ}$  30 C., in combination with a reserve, and subsequently treating the fabric with lye of ordinary temperature, and stretching it to obtain transparent patterns.

In testimony that I claim the foregoing as 35 my invention, I have signed my name in presence of two subscribing witnesses.

OSCAR KLAUSER.

Witnesses:

FRANK DINUNKE,  
EMIL WEILE.